# EUROPEAN PATENT SPECIFICATION

(11) **EP 1 786 988 B1**
(45) Date of publication and mention of the grant of the patent: **23.02.2011**
(21) Application number: 05771613.6
(22) Date of filing: 10.08.2005
(51) Int. Cl.: B28B 1/52, B28B 7/00, E04B 1/12, E04C 2/04

(54) **Full wall element of cement stabilised wood wool, method to produce it and building method using it**
Volles Wandelement aus zementstabilisierter Holzwolle, Verfahren zu seiner Herstellung und Bauverfahren zu seiner Anwendung
Élément de paroi pleine de laine de bois stabilisée au ciment, son procédé de fabrication et procédé de construction qui l'utilise

(30) Priority: 10.08.2004 SE 0401994
(43) Date of publication of application: 23.05.2007
(73) Proprietor: Ydre Träullsväggar AB, 570 60 Österbymo (SE)
(72) Inventor: RÜCKERT, Mattias, S-245 45 Staffanstorp (SE)
(74) Representative: Bengtsson, Peggy Katrin
(86) International application number: PCT/SE2005/001195
(87) International publication number: WO 2006/016844

(56) References cited:
- WO-A1-98/21422
- DE-U1- 7 914 865
- FR-A- 940 898
- GB-A- 416 223
- GB-A- 453 906
- GB-A- 628 335
- GB-A- 684 153
- GB-A- 750 127
- GB-A- 2 346 626

## Description

### Technical field

The present invention refers to a production method for wall elements of floor-to-floor height, which elements are cast from a mix of cement stabilised wood wool, to a construction element as per the preamble of claim 5, and a method for producing buildings as per the preamble of claim 11. Said production method, construction element and method for producing buildings are disclosed by document GB 750 127 A.

### Background of the invention

Cement stabilised wood wool today only exists in the form of so-called wood wool building slabs. This material, which is produced out of wood wool, cement and water, has been existing in Europe since the 1920s. The slabs are typically 500 or 600 mm wide and 2000 or 2400 mm long. The thickness varies between 20 and 150 mm. The wood wool building slab has primarily been used as plaster carrying wall isolation, sound absorbing ceiling and self-supporting ceiling insulation.

The material is characterised by good heat insulation capability and high thermal capacity. It possesses a great capability to store moisture and because of its open structure it can also rapidly absorb and release moisture. The wood wool building slab is not affected by rot and has a documented high resistance to mildew. Plastered wood wool building slabs have remained on frontages exposed to rain in over 50 years and also been buried in the ground for 30 years, without being affected. Further, the material possesses high fire resistance. The wood wool building slab does not emit any formaldehyde and negligible amounts of volatile organic compounds (VOC).

The present method of manufacturing wood wool building slabs is limited to a maximum thickness of 150 mm and a maximum width of 600 mm. This precludes manufacturing of wall elements in one single piece. Putting together wood wool building slabs into full wall elements is, in view of industrial engineering, relatively costly.

### Summary of the invention

The present invention refers to a method for producing construction elements with the aid of wood wool, cement and water comprising the following steps:
- arranging moulds for casting of the elements;
- taking wood wool and wetting it;
- stabilising the water content of the wood wool to 25%;
- mixing the stabilised wood wool with dry cement in a ratio by weight of 1:1.88 to 1:1.92;
- pouring the mix into the mould;
- letting the mix cure.

It also refers to a construction element for walls, comprising cement bound wood wool, characterised in that the element as a finished product has a density of 200 - 300 kg/m³.

The present invention further refers to a method for producing buildings comprising the following steps;
- attaching a construction element, as mentioned above, to the bedding with the aid of plaster;
- joining said elements sideways by casting a concrete column in the vertical cavities formed by means of chases provided in the sides of the elements;
- casting a capping piece of concrete in chases on the upper side of the element, the capping piece can be used to attach rafters.

### Brief description of the drawings

Fig 1 shows an example of a section of a steel mould (1.1) for casting a full wall element of cement bound wood wool. At the sides of the mould are triangular strips (1.2) arranged to produce the V-shaped chase at the ends of the element, according to fig 3.
Fig 2 shows an example of casting a full wall element in section. Two lifting straps (2.1), which are anchored to a round timber (2.2), are cast into the element. In the upper side of the mould is a tin plate (2.3) arranged to produce the rectangular chase, according to fig 4.
Fig 3 shows how the V-shaped chases (3.1) in the element ends forms a rectangular cavity (3.2) intended for an in-site cast concrete column which joins together the elements.
Fig 4 shows the rectangular chase (4.1) in the upper side of the wall elements, as well as how the wall elements are temporarily joined together by U-shaped tin plates (4.2).
Fig 5 shows an example of a completed full wall element with cut-out window openings in perspective, as well as how the elements are applied to the foundation.
Fig 6 shows a guiding rail of perforated panel (6.1.) attached to the concrete slab.
Fig 7 shows an example of how a wood wool element (7.1) is glued to the bedding using a cement-based plaster (7.2).
Fig 8 shows a joining of wood wool elements using concrete columns moulded on place (8.1). A dowel made of reinforcing iron is anchored in the foundation into the element joint (8.2).
Fig 9 shows how the capping piece is cast (9.1) into the upper side of the element as well as reinforced with reinforcing steel (9.2).
Fig 10 shows an example of securing devices (10.1) for windows and doors.
Fig 11 shows an example of securing a rafter into the capping piece by means of angle fittings (11.1) being attached to annular beam as well as the rafter. The underside of the rafter is protected by moisture barrier (11.2).
Fig 12 shows electric conduits and boxes (12.1) which have been milled into the masonry and thereafter repaired with plaster (12.2) before the surface layer is applied.
Fig 13 shows a section of a wall of wood wool elements, which has been surface treated using outside (13.1) and inside (13.2) reinforced plaster, as well as the wind-sealed plaster sludge on the crown of the wall (13.3).
Fig 14 shows a U-shaped beam (14.1) which is applied between two wall elements. The upper edge of the elements is notched (14.2) for placement of the beam.

### Detailed description of preferred embodiments

The invention refers on one hand to a production method for manufacturing outer wall elements of cement stabilised wood wool, i.e. full wall elements, and on the other hand of a construction system for putting together these elements to supporting outer walls. The thickness of the elements is selected based on desired heat insulation and supporting capability. The technique is primarily directed to walls that are not subjected to big vertical loads, e.g. outer walls in small buildings.

### Method of production

The wood wool elements are manufactured by casting a wood wool mass (a mixture of wood wool, cement and water) in steal moulds. The manufacturing of the wood wool mass is done in such a way that the wood wool mass, which is manufactured by spruce wood in a special plane, is moistened and thereby mixed with cement. In this connection, the mixing proportions between the cement and the moistened wood wool are significant for the elasticity of the mass upon casting: if too much cement is used, the mass of wood wool and cement does not become elastic enough, thus increasing the density. If, on the other hand, too little cement is used, the resistance might be to low. The mixing of the wood wool mass, as well as the filling of the moulds, differ from the manufacturing of the wood wool building slabs, which has a maximum thickness of 150 mm. Full wall elements, according to an embodiment of the present invention, are produced using a weight ratio between wet wood wool and dry cement of 1:1.9 (for conventional wood wool building slabs the mixing proportions are 1:2.0). This mixing ratio of 1:1.90 has been proven to manage a casting height of 400 mm without collapsing and becoming too compact, and the density can be varied from 200 kg/m³ to 300 kg/m³. Tests have shown that a mixing ratio of 1:1.88 can give rise to problems with the surface strength of the material. At mixing proportions of 1:1.92 some densities becomes too dense and collapses. Tests have also shown that there may arise problems at the lower mixing ratio getting all the wood wool covered with cement. It is important to get all wood wool covered with cement because the cement produces resistance against fire and microbial growth on the finished product. According to one embodiment of the invention, the moulds are 6 m long, 2.4 m high and 400 mm deep (inside measures), however, the measures can be adapted to the desired size of the wall elements. An adjustable tin plate having a cross section of 100 x 160 mm, is arranged adjacent of the upper end of the moulds, to create a chase in the upper edge of the elements. In a similar way, batters with triangular cross sections are arranged at both ends of the mould to create V-shaped chases in the sides of the elements. Lifting straps are cast in each side of the element to enable handling after curing and during assembly. In order to achieve the desired density, the wood wool mass is continuously weighted during the filling of the moulds. The wood wool mass is subsequently spread evenly over the surface of the lying mould, in order for an even density to be achieved. When all wood wool mass is distributed, the moulds are slightly over-filled. The mass is compacted by stacking the moulds on top of each other, the underside of the upper mould forming a lid for the mould lying below. On the top-most mould is placed a mould lid and on top of that concrete weights, weighing approximately 1.000 kg/m². Stripping is possible after 24 hours. Subsequently, the elements are raised and put to dry. The window openings, if any, are normally cut out after the elements are cured, but the elements can be moulded with holes for windows. Doors and large window sections are arranged between two wall elements. The upper edge of the wall elements is notched for storage to U-shaped beams according to fig 14. On both sides of the window- and door openings, mounting plates are arranged to support the fastening. In this mounting plate windows and doors can be attached using frame screw. The full wall elements can be delivered to the construction site as soon as they are cured to sufficient strength and dried out to the desired density. The ready-to-deliver elements hold a density of 200-300 kg/m³ (the exact density can vary between different buildings, primarily depending on desired heat insulation).

### Building system

For small houses, the walls of wood wool element are manufactured by way that the prefabricated elements are put directly on the foundation, normally on an edge beam. The elements are attached to the bedding by way of putting them in a string of plaster at the inside of the wall. When the elements are placed next to each other, a vertical cavity having a quadratic cross section with the side 70 mm, is formed through the V-shaped chases, see fig 3. The elements are temporarily kept in place by stamp and are mutually stabilised in the upper edge using U-shaped tin plates. The elements are laterally joined together by moulding concrete columns into the vertical cavities. Apart from joining the elements together, the concrete columns have the purpose of providing the wall with sufficient vertical load bearing capacity for elements with low density and for elements having a thickness down to 150 mm. Subsequently a concrete beam (as a capping piece/annular beam) with the height of 160 mm and the width of 100 mm, is moulded in the chase of the upper side of the elements. This beam is reinforced together with the concrete columns. The capping piece can also be made as a higher beam if it is necessary to distribute loads over large window sections. The rafters are anchored in the capping piece with aid of angle irons, alternatively moulded into the capping piece or attached by screws. The windows and doors are mounted, using ordinary frame screw and plug, into mounting plates, according to fig 10.

For inner surface treatment is used either plaster or gypsum wallboard. Plaster is preferably armed using welded armouring net made of galvanised, alternatively stainless, steel wire. The armouring reinforcement is placed in the outer plaster layer. On top of the element junctions an armouring net is placed also in the coarse stuff. In this way, a double armouring is produced over the element joints. In case gypsum wallboard is used, these are glued to the wall with gypsum plaster. The joints between the boards are filled by putting a string of gypsum plaster between the wood wool elements and the gypsum boards along the entire joint.

On the outside the surface treatment consists of plaster, which is armoured in the same way as the inside plaster, or any other type of facade material. The crown of the wall and the window openings are sealed against the wind using plaster sludge. If a not airtight facade material, such as wood panel or facade bricks is used, the outside of the brick work has to be air-tightened by sludging.

Electric wires are inserted into the masonry by milling groves (as for e.g. light concrete walls). Small load fixings to the wall, e.g. of paintings, is done in the plaster layer (alternatively the gypsum board) using plastic plugs, metal expansion anchors or rubber expansion anchors. In case of heavier load fixings, typically kitchen cupboards or wall-hanged book shelves, sheet metal profiles placed in slit/slotted groves in the wall, are used. As an alternative, screw plug or injection plaster can be used.

Further details of the construction system are apparent from the description of the figures below as well as from the patent claims.

In a further embodiment of the invention, the production method according to the present invention, moulds, according to fig 1, are used to cast full wall elements of cement-bound wood wool, according to fig 2. The elements are cast with chases in the side of the elements, according to fig 3, to enable a lateral joining of the elements. The elements are manufactured with a chase at the upper edge, in accordance with fig 4, to enable casting of capping pieces/annular beam. The window openings are cut out from the finished elements, see fig 5.

In the construction system according to the present invention, wood wool elements are placed on the bedding, in accordance with fig 6, towards a guiding rail made of perforated sheet metal according to fig 7, in a string of plaster. The elements are joined, in accordance with fig 8, by means of concrete columns cast in the joints between the elements. A capping piece is cast in concrete on top of the wall, according to fig 9, in such a way that it is reinforced together with the concrete columns. Windows and doors are attached with aid of frame screws in mounting rails of tin plate in accordance with fig 10. The rafters are mounted in the capping piece, according to fig 11.

The electric wires are inserted in the masonry, according to fig 12. Inside and outside plaster is arranged in accordance with fig 13. The plaster is to be reinforced with welded reinforcement net with galvanised, alternatively stainless, steel wire.

### Example

In still a further embodiment, a method for producing full wall construction elements comprises the steps of:
- providing wool wool; Wood wool having the following characteristics is preferred: spruce wood strips each having an approximate thickness of 0.3 mm, a width of 2.5 mm and a length of 300 mm;
- subjecting the wood wool for a water bath, thereby wetting the wood wool;
- subjecting the wet wood wool to rolling between rubber rolls thereby causing the wood wool to assume a uniform water content. Preferred water content is 24-26%, and more preferred 25% (by weight), when mixing with the dry cement;
- weighing the wood wool before and after the water bath;
- putting a measured amount of the wood wool from the rubber rolls in a container for mixing with dry cement. The amount of wood wool can, e.g., be measured using load measuring cells (Siemens, Germany);
- adding dry cement to the mixing container. The amount of dry cement is preferably 1.88-1.92 times the amount of wood wool with uniform water content, measured as weight ratio. Preferably is some kind of dispensing device used, e.g. from Thomal, to achieve a suitable dose of cement. The cement is preferably Standard Portland. A ratio of wood wool to cement of 1:1.90 or in the interval of 1:1.895 to 1:1.905, have shown to provide good properties to the finished elements;
- mixing the mix. During tests a Van Elten device (Dutch) has been used. Mixing was continued under 40-60 seconds;
- pouring the mix into moulds. The production can be performed at temperatures above zero. Tests were performed indoors in a hall.

## Claims

1. A method for producing construction elements (7.1) with the aid of wood wool, cement and water comprising the following steps:
a) arranging moulds (1.1) for casting of said elements;
b) taking wood wool and wetting it;
c) mixing the wood wool with dry cement in a ratio by weight of 1:1.88 to 1:1.92;
d) pouring the mix into the mould (1.1);
e) letting the mix cure, **characterised in that**
between steps b) and c) the method further comprises the step of stabilising the water content of the wood wool to 24-26%;
and **in that** in step c) the stabilised wood wool is mixed with dry cement in a ratio by weight of 1:1.88 to 1:1.92.

2. The method of claim 1, further comprising the steps of:
filling the mould (1.1) when it is laying down;
overfilling the mould (1.1) to some extent;
placing a number of moulds (1.1) on top of each other;
arranging a cover on top of the topmost mould (1.1);
arranging concrete weights on top of said cover weighing approximately 1.000 kg/m³_{.}

3. The method of claim 1, where said weight ratio of wood wool to cement is between 1:1.895 and 1:1.905.

4. The method of claim 3, where said weight ratio of wood wool to cement is 1:1.90.

5. A construction element (7.1) for walls, comprising cement-bound wood wool, where said element (7.1) is produced from a homogeneous mix of wood wool, water and cement, **characterised in that** said element (7.1), as a finished product, has a density of 200-300 kg/m³.

6. The construction element (7.1) according to claim 5, **characterised in that** a V-shaped chase (3.1) has been arranged in the side of said element (7.1) such that when two elements (7.1) are placed next to each other, a vertical cavity (3.2) is formed between the two elements (7.1).

7. The construction element (7.1) according to claim 6, **characterised in that** a rectangular chase (4.1) is arranged at the top of the element, useable as support for a concrete beam.

8. The construction element (7.1) according to claim 7, **characterised in that** said element (7.1) has a thickness of 150-400 mm.

9. The construction element (7.1) according to claim 8, **characterised in that** said element (7.1) has a height or a width of approximately 2.4 x 6.0 m.

10. The construction element (7.1) according to claim 9, **characterised in that** one or more window or door openings have been arranged in said element (7.1), and **in that** one or more fixing devices (10.1) are arranged on both sides of said opening(s).

11. A method for producing buildings comprising the following steps:
attaching a construction element (7.1) to the bedding with the aid of plaster (7.2);
joining said elements (7.1) sideways by casting a concrete column (8.1) in the vertical cavities (3.2) formed by means of chases (3.1) provided in the sides of the elements (7.1);
casting a capping piece (9.1) of concrete in chases (4.1) on the upper side of the element, said capping piece (9.1) can be used to attach rafters,
**characterised in that** said element (7.1.) is a construction element according to claims 5 -10.

12. The method of claim 11 further comprising the step of sealing said element (7.1) with plaster (13.1, 13.2).

13. The method of claim 12 further comprising the step of providing double layers of reinforcing nets in the surface plaster (13.1, 13.2) over the joint between two elements.

## Patentansprüche

1. Verfahren zum Erzeugen von Konstruktionselementen (7.1) mit Hilfe von Holzwolle, Zement und Wasser, umfassend folgende Schritte:
a) Anordnen von Gussformen (1.1) zum Gießen der Elemente;
b) Hernehmen der Wolle und Nässen dieser;
c) Mischen der Holzwolle mit trockenem Zement;
d) Schütten der Mischung in die Gussform (1.1);
e) die Mischung aushärten lassen
**dadurch gekennzeichnet, dass**
zwischen den Schritten b) und c) das Verfahren ferner den Schritt umfasst, den Wassergehalt der Holzwolle bei 24-26% zu stabilisieren und dass in Schritt c) die Holzwolle mit trockenem Zement in einem Gewichtsverhältnis von 1:1,88 bis 1:1,92 gemischt wird.

2. Verfahren nach Anspruch 1, ferner umfassend die Schritte:
Füllen der Gussform (1.1), wenn sie unten liegt;
Überfüllen der Gussform (1.1) bis auf ein gewisses Maß:
Platzieren einer Anzahl von Gussformen (1.1) aufeinander;
Anordnen einer Abdeckung auf der obersten Gussform (1.1);
Anordnen von Betongewichten auf der Abdeckung, die etwa 1000 kg/m³ wiegen.

3. Verfahren nach Anspruch 1, bei dem das Gewichtsverhältnis von Holzwolle zu Zement zwischen 1:1,895 und 1:1,905 liegt.

4. Verfahren nach Anspruch 3, bei dem das Gewichtsverhältnis von Holzwolle zu Zement bei 1:1,90 liegt.

5. Konstruktionselement (7.1) für Wände, umfassend zementgebundene Holzwolle, wobei das Element (7.1) aus einem homogenen Gemisch von Holzwolle, Wasser und Zement hergestellt ist,
**dadurch gekennzeichnet, dass**
das Element (7.1) als fertiges Produkt eine Dichte von 200-300kg/m³ aufweist.

6. Konstruktionselement (7.1) nach Anspruch 5, **dadurch gekennzeichnet, dass** ein V-förmiger Leitungskanal (3.1) so in der Seite des Elements (7.1) angeordnet ist, dass wenn zwei Elemente (7.1) nebeneinander platziert sind, eine vertikale Aussparung (3.2) zwischen den zwei Elementen (7.1) ausgebildet ist.

7. Konstruktionselement (7.1) nach Anspruch 6, **dadurch gekennzeichnet, dass** ein rechteckiger Leitungskanal (4.1) oben auf dem Element angeordnet ist, der als Lager für einen Betonbalken verwendbar ist.

8. Konstruktionselement (7.1) nach Anspruch 7, **dadurch gekennzeichnet, dass** das Element (7.1) eine Dicke von 150 - 400mm aufweist.

9. Konstruktionselement (7.1) nach Anspruch 8, **dadurch gekennzeichnet, dass** das Element (7.1) eine Höhe oder eine Breite von etwa 2,4 x 6,0 m aufweist.

10. Konstruktionselement (7.1) nach Anspruch 9, **dadurch gekennzeichnet, dass** ein oder mehrere Fenster- oder Türöffnungen in dem Element (7.1) angeordnet sind, und dass ein oder mehrere Befestigungseinrichtungen (10.1) an beiden Seiten der Öffnung(en) angeordnet sind.

11. Verfahren zum Erzeugen von Gebäuden, umfassend folgende Schritte:
Anbringen eines Konstruktionselements (7.1) auf die Lagerung mit Hilfe von Putz (7.2);
seitliches Verbinden der Elemente (7.1) durch Gießen einer Betonsäule (8.1) in vertikalen Aussparungen (3.2), die mittels Leitungskanälen (3.1) ausgebildet sind, die in der Seite des Elements (7.1) vorgesehen sind;
Gießen eines Haubenstücks (9.1) aus Beton in Leitungskanälen (4.1) an der oberen Seite des Elements, wobei das Haubenstück (9.1) zum Anbringen von Sparren verwendet werden kann,
**dadurch gekennzeichnet, dass**
das Element (7.1) ein Konstruktionselement nach einem der Ansprüche 5 - 10 ist.

12. Verfahren nach Anspruch 11, ferner umfassend den Schritt des Versiegelns des Elements (7.1) mit Putz (13.1, 13.2).

13. Verfahren nach Anspruch 12, ferner umfassend den Schritt des Bereitstellens von Verstärkungsnetzdoppelschichten in dem Oberflächenputz (13.1, 13.2) über der Verbindung zwischen zwei Elementen.

## Revendications

1. Procédé pour produire des éléments de construction (7.1) à l'aide de laine de bois, de ciment et d'eau comprenant les étapes suivantes consistant à :
a) agencer les moules (1.1) pour le moulage desdits éléments ;
b) prendre la laine de bois et la mouiller ;
c) mélanger la laine de bois avec du ciment sec ;
d) déverser le mélange dans le moule (1.1) ;
e) laisser le mélange durcir, **caractérisé en ce que** :
✔ entre les étapes b) et c), le procédé comprend en outre l'étape consistant à stabiliser la teneur en eau de la laine de bois à 24-26% ;
✔ et **en ce qu'**à l'étape c), la laine de bois stabilisée est mélangée avec du ciment sec selon un rapport en poids de 1:1,88 à 1:1,92.

2. Procédé selon la revendication 1, comprenant en outre les étapes consistant à :
✔ remplir le moule (1.1) lorsqu'il est posé ;
✔ remplir le moule (1.1) de manière excessive jusqu'à une certaine mesure ;
✔ placer un nombre de moules (1.1) les uns au-dessus des autres ;
✔ agencer un couvercle sur la partie supérieure du moule le plus haut (1.1) ;
**✔** agencer des poids en béton sur la partie supérieure dudit couvercle pesant approximativement 1000 kg/m³.

3. Procédé selon la revendication 1, dans lequel ledit rapport de poids de la laine de bois sur le ciment est compris entre 1:1,895 et 1:1,905.

4. Procédé selon la revendication 3, dans lequel ledit rapport de poids de la laine de bois sur le ciment est de 1:1,90.

5. Élément de construction (7.1) pour murs, comprenant de la laine de bois-ciment, dans lequel ledit élément (7.1) est produit à partir d'un mélange homogène de laine de bois, d'eau et de ciment, **caractérisé en ce que** ledit élément (7.1), en tant que produit fini, a une densité de 200-300 kg/m³.

6. Élément de construction (7.1) selon la revendication 5, **caractérisé en ce qu'**une chasse en forme de V (3.1) a été agencée dans le côté dudit élément (7.1) de sorte que lorsque deux éléments (7.1) sont placés l'un à côté de l'autre, une cavité verticale (3.2) est formée entre les deux éléments (7.1).

7. Élément de construction (7.1) selon la revendication 6, **caractérisé en ce qu'**une chasse rectangulaire (4.1) est agencée au niveau de la partie supérieure de l'élément, utilisable en tant que support pour une poutre en béton.

8. Élément de construction (7.1) selon la revendication 7, **caractérisé en ce que** ledit élément (7.1) a une épaisseur de 150-400 mm.

9. Élément de construction (7.1) selon la revendication 8, **caractérisé en ce que** ledit élément (7.1) a une hauteur ou une largeur d'approximativement 2,4 x 6,0 m.

10. Élément de construction (7.1) selon la revendication 9, **caractérisé en ce qu'**une ou plusieurs ouvertures de fenêtre ou porte ont été agencées dans ledit élément (7.1), et **en ce qu'**un ou plusieurs dispositifs de fixation (10.1) sont agencés sur les deux côtés de ladite (desdites) ouverture(s).

11. Procédé pour produire des bâtiments comprenant les étapes suivantes consistant à :
✔ fixer un élément de construction (7.1) sur l'assise à l'aide de plâtre (7.2) ;
✔ assembler lesdits éléments (7.1) latéralement en coulant une colonne de béton (8.1) dans les cavités verticales (3.2) formées au moyen des chasses (3.1) prévues dans les cotés des éléments (7.1) ;
✔ couler une pièce de chapeau (9.1) en béton dans les chasses (4.1) sur le côté supérieur de l'élément, ladite pièce de chapeau (9.1) peut être utilisée pour fixer les chevrons,
**caractérisé en ce que** ledit élément (7.1) est un élément de construction selon les revendication 5 à 10.

12. Procédé selon la revendication 11 comprenant en outre l'étape consistant à sceller ledit élément (7.1) avec du plâtre (13.1, 13.2).

13. Procédé selon la revendication 12, comprenant en outre l'étape consistant à prévoir deux couches de filets de renforcement dans le plâtre de surface (13.1, 13.2) sur le joint situé entre les deux éléments.
